

April 16, 1929.

A. H. SPALDING ET AL  
HALFTONE PHOTOMECHANICAL PRINTING PLATE  
AND METHOD FOR PRODUCING THE SAME  
Filed Sept. 19, 1925

1,709,327

FIG. 1



FIG. 2



FIG. 3



FIG. 4



FIG. 5



FIG. 6



FIG. 7



FIG. 8



FIG. 9



A. H. Spalding INVENTORS  
J. M. Chandakian  
BY  
John D. Morgan ATTORNEY

## UNITED STATES PATENT OFFICE.

AMOS H. SPALDING, OF MANHASSET HILLS, AND JAMES M. CHANKALIAN, OF NEW YORK, N. Y., ASSIGNEES TO POWERS PHOTO-ENGRAVING COMPANY, A CORPORATION OF NEW YORK.

HALFTONE PHOTOMECHANICAL PRINTING PLATE AND METHOD FOR PRODUCING THE SAME.

Continuation of applications Serial No. 583,910, filed August 23, 1922, and Serial No. 733,058, filed August 20, 1924. This application filed September 19, 1925. Serial No. 57,274.

The invention relates to a novel process for making half-tone printing plates, and in certain aspects thereof it relates more especially to a process for making such plates 5 for use in making stereotyped plates or electro-type plates.

The distinctive objects and advantages of the invention will be set forth hereinafter in part, and in part will be obvious herefrom, 10 or may be learned by practicing the invention.

The invention consists in the novel articles, step or steps, sequence of steps and processes herein described.

15 This application is a continuation of our two earlier and copending applications, Ser. No. 583,910, filed August 23, 1922 and Ser. No. 733,058, filed August 20, 1924.

20 The accompanying drawings are diagrammatic in character, as the actual surfaces and parts are microscopic. They will be explained and referred to later in the specification.

25 The invention is directed to providing a process for making half-tone printing plates which will have superior printing properties, will correctly and uniformly produce the varying tones of the original, and which shall be especially adapted for making matrices for casting stereotype plates and wax 30 molds for making electrotype plates.

The process produces plates having the merits or advantages described by reason of the form or structure of the screen figures 35 of the plate, that is, plates having in the shadows clean, clear, open cells or depressions of practically the depth between the dots, or other screen figures, in the lighter and lightest tones. Such plates also have 40 the screen figures, including the dots in the lightest tones with sharp pointed edges and with smooth downwardly and outwardly sloping sides. There is also a uniformity of tone throughout a given tone, due to the uniformity of the shape of the dots or equivalent 45 screen figures.

The invention finds one of its widest and most important applications in the making of zinc half-tone plates for use in making 50 stereotype plates, as in newspaper printing, and the exemplary manner of carrying out the process is hereinafter described in the

production of such a plate; although it will be understood that the invention is likewise applicable to the making of other kinds of 55 half-tone printing plates.

In the making of half-tone plates in newspaper work, great rapidity is imperative, as frequently but a few minutes are available from the time a photograph is received until 60 the matrix must be delivered to the stereotype room. Irrespective, however, of the speed of production, the half-tone plates must be of such high quality and peculiar and characteristic properties as to permit 65 a perfect matrix to be made therefrom, and then from the matrix stereotype plates which will give excellent results even under the difficult conditions of newspaper printing.

For certain reasons, among which are the 70 great speed at which newspaper half-tones must be produced, and the relatively great depth required in the etched half-tone plate, it is customary and desirable to give several etchings or "bites" to the plate. One of the 75 principal faults in half-tone plates, especially in zinc plates, which are etched at great speed and to the required great depth for newspaper stereotyping, is the action of the etching fluid in "undercutting". This is 80 due to the fact that the acid or etching fluid not only corrodes or eats away the metal vertically but also laterally. In a properly made half-tone negative for newspaper illustration, all the transparent dots, as well 85 as the areas representing the half-tones are much wider than intended in the final result. This is because of the allowance which must be made for the lateral corrosion of the acid or solution used in etching the plate, the 90 action of the acid as is well known being lateral as well as downward.

The positive photographic prints made from such negatives on the zinc plates, in an acid-resisting material is much stronger 95 than required, to make allowance for this lateral etching. This lateral etching causes the undercutting and creates shoulders or irregularities in the sides of the dots, or other screen figures, and creates difficulty 100 and damage in withdrawing the matrices from the finished half-tone plate in stereotyping, and the wax mold in electrotyping. The impurities present in the metal of the

plate, and which usually resist the acid, also contribute to the roughness of the screen figures constituting the design.

By creating the screen figures in the half-tone plate with true and well-defined edges for their top surfaces, and smooth downwardly and outwardly supporting sides, the matrix or the wax mold may be withdrawn from the plate without in any wise marring or distorting the impression made in the matrix or wax mold by the half-tone plate.

By the usual process it is generally found that one etching of the developed plate does not give the requisite depth, and further-  
more when the plate is etched twice, while sufficient depth is secured, the dots or screen figures for the high lights and lighter tones will be formed with shoulders or heads. This is due to the dragon's blood powder or other resist running partly down the sides of the dots or screen figures formed by the first etch, the etching fluid then acting only on the bottom parts of the sides of the dots or other screen figures. At the same time, the second etch has no effect upon the middle tones and deep shadows for the reason that the dragon's blood or other resist has practically entirely filled the depressions made by the first etch.

Furthermore, the re-etching of the plate tends to produce ragged and irregularly formed dots or other screen figures due to the adherence to the side wall of the screen figures of the powder of dragon's blood, or other resist, in more or less granulated or disintegrated form and scattered or disposed irregularly adherent on the side walls of the dots or other screen figures.

In carrying out our process, in the present preferred commercial practice thereof, a metal plate, such as a zinc plate is coated with a light-sensitive coating, and preferably with an "enamel" coating, such as the well-known enamel consisting of a solution of glue, white of eggs and ammonium bichromate.

After this enamel coating is baked on the plate, it receives the usual exposure through the screen negative. Thereafter the exposed plate is "developed," usually with cold water, and thereafter a suitable hardener is applied to the developed coating, such as a solution of chromic acid, alum, ammonium bichromate and water. It is also a common practice to stain the coating with an aniline dye. The foregoing steps are well-known and are usually practiced in the art and may be employed in any form or manner best adapted or most suitable as desired.

In the further preparation of the plate by our process, it receives preferably a preliminary, or repeated preliminary etchings, and then a final etching which produces a plate having adequate and usually and preferably equal depth in the depressions be-

tween the screen figures in all parts of the plate, and having screen figures which are true and symmetrical in form, and having smooth side walls which are downwardly and outwardly inclined. The screen figures have the surface and the side walls thereof very smooth, uniform and true and without the irregularity and raggedness commonly resulting from the usual or ordinary process of plate making.

The first preliminary etch, applied preferably to a baked enamel plate, when zinc is used, may be a dilute nitric acid, say in the proportions of one part acid to twenty parts water, the etch being applied usually from twelve to fifteen seconds, although all of these may be varied as desired, so far as concerns the main features of the present invention.

After the etching has been completed, the plate is washed and dried and is then powdered "four ways" with the dragon's blood or other resist, and is preferably baked after each way of powdering so that the resist will run down and become attached to the sides of the dots to protect them from the action of the next etch.

The next etch is generally similar to the first etch, using the same kind and strength of acid, but the plate is usually etched from thirty to forty-five seconds, although all these steps may be varied to suit the particular case or work. The plate is then washed, preferably with an alkaline solution, such as a caustic soda solution which will thoroughly clean the plate down to the enamel.

The plate as so prepared, or otherwise properly prepared, is subjected to the action of a strong or a pure acid, that is, for example, nitric acid of full commercial strength, which is applied by means of a suitable brush, such as a glass brush or one of pig's bristles, the acid being applied by brushing in all directions, and this is usually and preferably continued until the high light dots reach their extreme point or become absolutely sharp, and the light tone dots proportionately so, and the depressions between the dots of the middle tones and in the shadows are formed into clean-walled, open cells equal in depth to the depressions between the high light dots. The acid as so applied to the plate has a uniform action throughout, the side walls of the dots, or other figures of the etched plate, being free from adhering powder and the tendency of the strong acid is to avoid undercutting. The high light dots also reach their extreme point, that is, are reduced to a minimum of area while, if so desired in particular cases, maintaining their height in the general level of the plate. The enamel also retains or remains on the surface substantially intact or unimpaired, as compared to the action

of the weaker or greatly diluted acids, as the water in the latter has a strong solvent effect upon the enamel.

Considering the invention next from the standpoint of the structure and structural steps and changes effected in the plates:

In Fig. 1 a glass screen figure negative 1 is diagrammatically shown, with light-obstructing parts 2 and light-transmitting parts 3.

After this enamel coating is dried on the plate, it receives the usual exposure to the screen-figure negative. Thereafter the exposed plate is developed, usually with cold water, or with alcohol if it is "cold enamel". It is also a common practice to stain the coating with an anilin dye. These steps are well known and usually practiced in the art, and may be employed in any form or manner best adapted or most suitable for the particular work and kind of plates being made.

In Fig. 2 a metal plate 6 is diagrammatically shown having a design thereon formed by the development of its enamel light-sensitive surface after exposure under the negative 1. The parts 7 are acid resistant enamel and define the design and effect the tone gradations, and the parts 8 are the parts of the metal bared by the development in the usual manner.

As previously stated, it is usually customary or desirable to give the plate a plurality of etchings or "bites", usually three or four, although the exact number is not essential. The first etching is for a short period in a weak acid solution, which may be dilute nitric acid, say in the proportion of one part acid to twenty parts water, this etch being applied usually from twelve to fifteen seconds, although the mixture and time may be varied as found desirable, so far as concerns the main features of the present invention.

As previously stated, this etch eats out the metal unprotected by the developed enamel surface constituting the design. It eats not only downwardly but also laterally slightly beneath the edges of the protective enamel coating. The result is that each isolated dot is corroded or eaten away on the sides, or "undercut" as it is termed, and is somewhat rough on its edges. This undercutting takes place on the edges of the design, and of all the areas protected on their surfaces by an acid resist.

Fig. 3 is a diagram of the plate at this stage, the undercuttings being shown at 9.

To prevent further undercutting in this same region during the second etching, and to greatly minimize the total undercutting by the successive etches or bites, an acid resist, usually a resinous powder or dragon's blood is applied to the sides of the screen figures so far as created by the first etching.

To cause this acid-resisting material to adhere all over the sides of the screen figure dots, the plate is usually "powdered" four ways, and is heated or baked preferably after every powdering.

When the sides of the screen figures are thus protected (as shown at 10 in Fig. 4), the plate is again etched, and this may be done with the same etching fluid, but in present preferred practice the etching is continued for a somewhat longer time, say from thirty to forty-five seconds, although it will be understood that practical details may be varied as desired. As before, the etching fluid acts both downwardly and laterally. However, due to the protection of the sides of the screen figures (as diagrammatically shown at 10), the area of this lateral corrosion by the second etching is both greatly circumscribed and is localized or limited both downwardly and outwardly from the surface of the screen figure (as diagrammatically shown at 12, Fig. 5), the areas acted upon by the first etching having been protected, as stated, from the action of the second etching solution by the resist 10.

In the case of a third etching, or any number of further etchings, this same step is repeated. That is, the portion on the sides of the screen figures which were affected by the undercutting action of the second etch are protected by an acid-resisting material in the manner previously described. Thus the portions undercut by the second etch are protected from the action of the third etch, and the undercutting action of the third etch is thus both circumscribed and localized, and occurs only in a relatively still smaller area and both farther down and farther out with respect to the sides of the screen figure.

The second "powdering" is shown in Fig. 6 and the third etching in Fig. 7, and the undercutting therefrom in Fig. 8 (all diagrammatically).

When sufficient depth between the screen figures, and especially between the high light dots have been effected, the resinous powder or other resistant material, adherent upon and protecting the sides of the dots or other screen figures is removed by a proper solvent, but the enamel coating or equivalent acid resisting material 7 is left adherent upon the tops of the screen figures, that is, upon the printing surface of the plate. The acid resist is removed by any suitable agent, an alkaline solution, such as a caustic soda solution, being usually employed.

The cleaned plate with the steps or shoulders formed on the sides of the screen figures is shown diagrammatically in Fig. 8.

On examination of the etched plate, it will be found that the high light dots are not as fine as they should be and the highest light dots could be brought to sharp points nor

are the small cavities in the shadows deep and wide enough. The principal fault, however, with the etched plate at this stage is, that on the sides of each dot, line or other screen figure, there is a series of steps or shoulders, each of these being slightly undercut. These ragged edges and sides of the dots, particularly the undercut side surfaces, interfere with and prevent the taking 10 of a proper papier-mâché mold for stereotyping for a wax mold for electrotyping. Not only are the screen figures ragged and rough, but they tear and deform the impression in the mold as it is withdrawn from the 15 plate after the impression has been made.

By our invention the rough edges of the etched screen figures are made regular and clean-cut, and the side faces of the screen figures are made smooth and outwardly and 20 downwardly sloping, by the elimination of the irregularities due to the undercutting. Also the etching is deepened in all parts of the plate or locally where desired, and the highest light dots are brought to sharp 25 conical points. The dots in the highest lights are brought, in some plates, to sharp points, and these points may be very slightly below the general plane of the plate surface, as shown at the right in Fig. 9. When the 30 high light dots are very slightly below the general surface of the plate, valuable advantages are realized for some kinds of work, as for instance less pressure in the press, longer wear of the plate, and brighter 35 high lights are secured. The plate is also better adapted for producing better results in stereotyping. There is thus produced a half-tone plate with increased contrast for newspaper printing, as well as having the 40 other desirable and advantageous characteristics set forth. The invention further provides for doing this very expeditiously, as is required in certain classes of work, such as newspaper work, as already described.

45 This is done, in the present preferred procedure, by brushing over the whole plate, which is now protected only by the enamel adherent upon its surface, with a strong acid, a pure acid being preferred, as for 50 example, nitric acid of full commercial strength. This is preferably applied by means of a suitable brush, such as a glass brush, or one of pig bristles, the acid being applied by brushing in all directions.

55 This will remove quickly the rough steps and shoulders on the sides of the dots or other screen figures, will deepen the shallow cavities in the shadows, will deepen and widen the etching between the lines and dots of 60 the whole plate and bring the dots in the high lights to still finer points, and the highest light dots to sharp conical points. Thus all the screen figures in the half-tone plate have firm clear edges, and the depressions 65 between the dots of the middle tones and in

the shadows are formed into clean-walled, open cells equal in depth to the depressions between the high light dots. One of the valuable features or effects of the process is to render coniform all the raised dots in the 70 plate and the sloping of all the sides of the lines in place of the rough, undercut steps and shoulders which were left after the several etchings.

This vigorous treatment produces an 75 etched plate with deeper, wider and smoother cavities between the dots, or other screen figures, which permit the forcing of a soft papier-mâché flung down into the deepest portions of the half-tone plate and allows 80 the withdrawal of the matrix without injury, and the same is true of the wax mold, which would be impossible if the impressions were taken with all the rough edges and the undercut steps and shoulders unremoved. It 85 will be understood that this treatment may be applied to the entire surface of the plate or locally, wherever desired, but usually it will be applied over the entire plate and then frequently it will be further applied 90 locally.

From the standpoint of the physical and chemical agencies, changes and processes involved and occurring, to the best of our present knowledge, the nature and operation 95 of our invention is substantially as follows:

Considering the plate after it has been exposed and developed, and the acid resist applied thereto, the high light portions of the design consist of spots or cones of the resist surrounded by the unprotected metal of the surface of the plate. The shadows of the design appear as a coating of resist with tiny holes in it, the bottom of these holes being the unprotected metal. The various 100 gradations of middle tones between the high lights and deep shadows are variously and proportionately intermediate in form between these two, that is, between the islands 105 of resist with the intervening bare metal of the plate in the high lights, and the uniform coat of resist with the small holes therethrough in the deep shadows.

Considering the surface of the plate from a somewhat different standpoint, the shadows may be considered as a coating of resist with capillary holes therethrough down to the metal surface of the plate, while the high light portions of the plate show very largely unprotected metal with a relatively small 110 proportion of the surface thereof protected by the dots or islands of resist. In these high light areas, the openings through the resist to the metal surface of the plate are of sufficiently large dimensions to eliminate 115 the effects that are associated with or are present with holes of capillary size, such as exist in the shadows. There will be a gradation in the middle tone from these free or non-capillary openings of the high lights to 120 125 130

the capillary openings in the shadows, proportionately to the degree or density of the different gradations of the intermediate tones.

In etching this surface of the plate with a given concentration of dilute acid, the following may be considered to be a fair picture of what occurs. In the high lights the exposed metal is etched freely and uniformly by the acid applied thereto, and the solution of the salt resulting from the chemical action, as a dilute acid solution, runs freely away. In this part of the plate it is believed that capillary action plays a negligible part, if present at all, because the distances between the cones or islands of resist are relatively great, and this is especially so when the coarser half tone screens have been used in making the negative.

In the deep shadows, on the other extreme, capillary portions play an important part. The dilute etching acid enters the holes or capillary openings in the resist and comes into contact with the exposed metal at the bottoms of these openings. Capillary action tends to hold the dilute acid, which is the product of the etching action, in the hole. There is thus not the free removal of the products of the reaction, as in the case of the etching of the high light areas as already described, where capillary action does not enter appreciatively into the process. In the shadow areas, capillarity draws the fresh acid in, and after the etching operation has begun, the action or force drawing in the acid is counter-acted by this same capillary attraction tending to hold the spent solution in the hole.

In the variously gradated middle tones, where the openings vary from slightly larger capillary openings up to the free openings representing a large proportion of the local area, the chemical action is similarly gradated and approximately in corresponding proportions.

As a consequence of these facts, conditions and physical and chemical actions, the actual amount of etching is greatest in the high lights, gradating decreasingly through the middle tones to the least amount in the shadows. This is manifested in the area of etch, or etching action, but is manifested more especially in the depth of the etching action. The relative amount of etch per unit surface, for illustration, may be given arbitrary numbers which would symbolize relative depths of etch. In a given case these may be 60, 25 and 15 for high light, middle tone and shadows, respectively.

To change this ratio of etch, it is only necessary to change the effective driving capillary force. For instance, if it is desired to decrease the etch in the shadows, the etching solution should have a surface tension such that it will enter less readily into

the capillary. This may be accomplished by using a more concentrated acid, which has a surface tension considerably lower than a more dilute solution of the acid. Having a lower surface tension, it has less tendency to go into the capillary, and therefore it etches less.

The high lights, however, are not so affected, since capillarity is negligible or of very little importance in the high light areas. The gradation and action in the middle tones would vary correspondingly and approximately proportionately. Thus by the use of strong acid it has been found that most of the etching is done in the high light. For example, and again using arbitrary numbers for a given case, the ratio of etching in the various areas may become say 85, 10 and 5, from the high lights, through the intermediate tones to the shadows.

It is probable that viscosity of the strong acid may also play a part in this action, as strong acid is more viscous than dilute. It would be harder to get the more viscous solution into the smaller hole and, therefore, the etching would be less in the shadows relatively to the high lights.

This etching action of the strong acid is apparent more especially in depth than in extent. In this it is different from the dilute acid etch. This is occasioned probably, to the best of our present knowledge and observation, by the fact that the gas evolved during the reaction tends to escape at the juncture of the acid and of the metal cones, protected by the patches of resist, which constitute the high light areas of the plate. The gas must escape in order that the etching may go on.

It would not push through the liquid between the cones or screen figures, for it can more easily escape at the contact surface with the metal cones or screen figures. Now, granting a uniform action over the whole surface, all of the gas from the reaction must pass the surface of the metal where the resist lies. Take a point on the plate in the bottom between two cones or screen figures in the high light, only the gas generated by the local etch tends to protect this surface, while this and all the remainder of the gas generated by surfaces between the middle point on the side of the cone or screen figure and the top thereof must pass a point at the surface of the metal plate, that is, the top of the cone beneath the layer of resist.

This gas tends to blanket the metal and to prevent the acid coming in contact with it. As this blanketing is least at the middle point between the cones or screen figures, it follows that the etching action will be greatest at such middle point. Consequently the etching action is manifested more in depth than in area, as compared with a dilute acid etch, which is relatively slow

and in which gas evolution is not such a factor.

The gases evolved in the case of the strong acid are principally oxides of nitrogen mixed with some hydrogen; while in the case of the dilute acid hydrogen is the principal gas evolved. The top of the cones of metal or screen figures of the plate may also be protected by local passivity, due to the action of the excessive amounts of oxide of nitrogen.

There is no tendency to undercut the resist, for as rapidly as the metal is etched away along the side and top of the cones or screen figures, the strong acid fumes, being oxidizing, eat away the resist. With dilute acid, however, this would remain as a shelf extending over the cone, occasioned by the metal having been dissolved from under the fringe of the resist path or dot.

The final result of the strong acid etch, or re-etch is a shifting of the relative amount of metal etch toward the high lights, occasioned by a decrease in the force driving the acid into the capillary, which decreases the relative amount of etch in the areas where capillarity is important, that is, in the middle tones and increasingly into the shadows. This ratio is changed, in the arbitrary example heretofore given, say from 60, 25 and 15 to 85, 10 and 5.

There is also a shifting in the extent of the etch, especially in the high lights to depth of etch alone, rather than depth and extent laterally of the plate. Added to this, there is a uniform oxidation of the fringe of resist, thus preventing shelving or so-called undercutting.

This application is a continuation of our applications Ser. No. 583,910, filed Aug. 23, 1922, and Ser. No. 733,058, filed Aug. 20, 1924. The practical shop method has been continuously and very widely and successfully in commercial use since some little time prior to the filling of the earlier application, and the practical use of the process is fully disclosed herein, the actual commercial plates produced possessing all the commercial excellencies and advantages described.

The physical and chemical facts, conditions and actions which have been added by way of elaboration and explanation, are observed with considerable difficulty owing to the microscopic minuteness of structure of the surface of the plate and the rapidity of the various actions, which occur beneath and are largely obscured by the etching fluids. However, the added explanatory matter represents our best present knowledge of what actually occurs during the process, from the physical and chemical standpoint; but it will be understood that the invention as a valuable and active commercial improvement is not limited or bound by the physical

or chemical theories and explanations given.

It will be understood that the various proportions, specific reagents and other details do not limit the invention; but that departures may be made from the details, within the scope of the accompanying claims, without departing from the principles of the invention and without sacrificing its chief advantages.

What we claim is:

1. The process of making a half-tone printing plate which comprises sensitizing a plate, exposing the plate to light through a toned screen-figure negative, applying a preliminary etch, applying a resist so as to leave the sides of the screen figures exposed, and etching the plate to deepen it while producing points with smooth downwardly and outwardly sloping sides, to effect a desired relation of the various tones of the half-tone plate.

2. The process of making a half-tone printing plate which comprises sensitizing the surface of a plate, exposing said surface through a half-tone screen figure negative, etching the plate and protecting the tops only of the tone-producing screen figures and leaving the sides thereof entirely unprotected, and re-etching the plate, thereby producing screen figures with smooth downwardly and outwardly sloping sides, to effect a desired relation of the various tones of the half-tone plate.

3. The process of making a half-tone printing plate which comprises sensitizing the surface of a plate, exposing said surface through a half-tone screen figure negative, etching the plate and repeatedly etching with a weak acid a plate having a surface of tone-producing screen figures, having a resist thereon and finally etching the plate with a strong acid without a resist, to effect a desired relation of the various tones of the half-tone plate.

4. The process of making half-tone printing plate which comprises applying a light-sensitive enamel layer to a plate, exposing the plate to light through a half-tone screen figure negative, etching the plate, removing the residue of the resist and etching the plate with only its residual enamel as a protection, to effect a desired relation of the various tones of the half-tone plate.

5. A half-tone printing plate having an enamel top surface with a great number of minute screen figures representing the corresponding tones of the original and with smooth downwardly and outwardly sloping sides entirely bounding the respective figures.

6. A half-tone printing plate having an enamel top surface with a great number of minute screen figures representing the corresponding tones of the original and in the high lights uniformly reduced to points and

in the shadows of uniform tone value with the intervening depressions clean and clear and with smooth sides entirely bounding the respective figures.

5 7. The process of producing a half-tone plate which comprises placing a light-sensitive enamel layer on a plate, exposing the plate to light through a half-tone screen figure negative, and etching the plate

10 including the steps of localizing the undercutting entirely about the separated screen figures by repeated etching, and then removing the resultant roughnesses from the sides of the screen figures of the plate, to effect 15 a desired relation of the various tones of the half-tone plate.

8. The process of producing a half-tone plate which comprises placing a light-sensitive enamel layer on a plate, exposing the 20 plate to light through a half-tone screen figure negative, and etching the plate including the steps of localizing the undercutting entirely about the separated screen figures by repeated etching, and then removing the 25 resultant roughnesses from the sides of the screen figures of the plate by the application of a strong acid, to effect a desired relation of the various tones of the half-tone plate.

9. The process of producing a half-tone 30 plate which comprises placing a light-sensitive enamel layer on a plate, exposing the plate to light through a half-tone screen figure negative, and etching the plate by a plurality of bites and protecting the undercutting entirely about the separated screen 35 figures made by one bite from the action of a succeeding bite, and removing the resultant roughnesses from the sides of the screen figures of the plate, to effect a desired 40 relation of the various tones of the half-tone plate.

10. The process of producing a half tone plate which comprises etching the plate by a plurality of bites and protecting the 45 undercutting made by one bite from the action of a succeeding bite, and removing the resultant roughnesses from the sides of the screen figures of the plate by scrubbing the plate with strong acid.

50 11. The process of producing a halftone plate which comprises creating an enamel design on the surface of the plate, etching the plate by a plurality of bites, and protecting the undercutting made by one bite from the 55 action of a succeeding bite, and removing the resultant roughnesses from the sides of the screen figures of the plate by scrubbing the surface of the plate with acid with all resist removed except the surface enamel.

60 12. A half tone printing plate having the high light dots with smooth conical sides terminating in points very slightly below the plane of the surface of the plate.

65 13. The process of producing a half-tone printing plate which comprises sensitizing

the plate with an enamel layer, exposing the plate to light through a half-tone screen figure negative, repeatedly etching the plate entirely about the separated screen figures, with solutions having varying surface tensions to regulate the relative depth and lateral extent of the different etches, to effect a desired relation of the various tones of the half-tone plate.

70 14. The process of producing a half-tone printing plate which comprises sensitizing the plate with an enamel layer, exposing the plate to light through a half-tone screen figure negative, repeatedly etching the plate entirely about the separated screen figures, 75 with solutions of differing degrees of viscosity to regulate the relative depth and lateral extent of the different etches, to effect a desired relation of the various tones of the half-tone plate.

80 15. The process of producing a half-tone printing plate which comprises sensitizing the plate with an enamel layer, exposing the plate to light through a half-tone screen figure negative, repeatedly etching the plate 85 entirely about the separated screen figures, with solutions, and varying the character of a succeeding etching solution to secure depth of etch with practically no lateral etch.

90 16. The process of producing a half-tone printing plate which comprises applying a light-sensitive layer to the surface of the plate, exposing and developing the plate to create screen figures thereon, preliminarily etching the plate with dilute acid, and subsequently etching the plate with strong acid 95 without a resist being applied preliminary to said etching.

100 17. The process of producing a half-tone printing plate which comprises applying an enamel light-sensitive layer to the surface of the plate, exposing and developing the plate, to create screen figures thereon, baking the developed enamel coating, preliminarily etching the plate with dilute acid, 105 and subsequently etching the plate with substantially undiluted acid without a resist being applied preliminary to said etching.

110 18. The process of producing a half-tone printing plate which comprises applying a light-sensitive layer to the surface of the plate, exposing and developing the plate, to create screen figures thereon, preliminarily etching the plate with dilute acid, applying 115 a resist to the surface of the plate, etching the plate with a dilute acid, and subsequently etching the plate with strong acid without a resist being applied preliminary to said etching.

120 19. The process of producing a half-tone printing plate which comprises applying an enamel light-sensitive layer to the surface of the plate, exposing and developing the plate, to create screen figures thereon, baking the developed enamel coating, pre- 125

liminarily etching the plate with dilute acid, applying a resist to the surface of the plate, etching the plate with a dilute acid, and subsequently etching the plate with strong acid 5 without a resist being applied preliminary to said etching.

20. A half-tone printing plate having its screen figures in the high lights uniformly reduced to points and in the shadows of uniform tone value with the intervening depressions clean and clear and with smooth sides.

21. The process of producing a photo-mechanical printing plate which comprises 15 applying a light-sensitive layer to the surface of the plate, exposing the plate through a half-tone screen-figure negative and developing the plate, preliminarily etching the plate with dilute acid, and subsequently 20 directly applying a strong etching acid by frictional means applied on the surface of the plate.

22. The process of producing a photo-mechanical printing plate which comprises 25 applying a light-sensitive layer to the surface of the plate, exposing the plate through a half-tone screen-figure negative and developing the plate, preliminarily etching the plate with dilute acid, and subsequently 30 directly applying a strong etching acid directly to all parts of the design except the faces of the screen figures.

23. The process of producing a photo-mechanical printing plate which comprises 35 applying a light-sensitive layer to the surface of the plate, exposing the plate through a half-tone screen-figure negative and developing the plate, applying an acid resist to the developed surface of the plate, pre- 40 liminarily etching the plate with dilute acid, and subsequently directly applying a strong etching acid to the plate.

24. The process of producing a photo-mechanical printing plate which comprises 45 applying a light-sensitive layer to the surface of the plate, exposing the plate through a half-tone screen-figure negative and developing the plate, applying an acid resist to the developed surface of the plate, pre- 50 liminarily etching the plate with dilute acid, and subsequently directly applying a strong etching acid by frictional means applied on the surface of the plate.

25. The process of producing a photo-mechanical printing plate which comprises 55 applying a light-sensitive layer to the surface of the plate, exposing the plate through a half-tone screen-figure negative and developing the plate, applying the acid resist to the developed surface of the plate, pre- 60 liminarily etching the plate with dilute acid, applying an acid resist to the etched surface, etching the plate with a dilute acid, and subsequently directly applying a strong 65 etching acid to the entire surface of the de-

sign on the plate except the faces of the screen figures.

26. The process of producing a photo-mechanical printing plate which comprises applying a light-sensitive layer to the surface of the plate, exposing the plate through a half-tone screen-figure negative and developing plate, preliminarily etching the plate with dilute acid, and subsequently directly applying a strong etching acid to the plate with the sides of the screen figures unprotected by any resist.

27. The process of producing a half-tone printing plate which comprises applying an enamel to the surface of the plate to 80 create screen figures thereon, exposing and developing the plate, preliminarily etching the plate with dilute acid, removing all resist except the enamel, and subsequently 85 etching the plate with strong acid without a resist being applied preliminary to said etching.

28. The process of producing a half-tone printing plate which comprises applying a light-sensitive enamel coating to the plate, 90 exposing the plate through a half-tone screen figure negative, applying a resist to the plate, and etching and cleaning the plate with a strong acid to insure the removal of all resistant matter except the enamel 95 surface of the plate.

29. The process of producing a half-tone plate to be used alone in printing, which comprises the steps of exposing a light-sensitive plate through a half-tone screen 100 figure negative to truly reproduce the light tones of the original, repeatedly etching the plate, localizing the undercutting by repeated etching, and then removing the resultant roughnesses from the sides of the 105 screen figures of the plate.

30. The process of producing a half-tone plate to be used alone in printing which comprises the steps of exposing a light-sensitive plate through a half-tone screen 110 figure negative to truly reproduce the light tones of the original, repeatedly etching the plate, localizing the undercutting by repeated etching, and then removing the resultant roughnesses from the sides of the 115 screen figures of the plate by the application of a strong acid.

31. The process of producing a half-tone plate to be used alone in printing, which comprises the steps of exposing a light-sensitive plate through a half-tone screen figure negative to truly reproduce the light tones of the original, repeatedly etching the plate, localizing the undercutting by repeated etching, and then removing the resultant roughnesses from the sides of the 120 screen figures of the plate by scrubbing the 125 plate with acid.

32. The process of producing a half-tone plate to be used alone in printing, which 130

comprises exposing a light-sensitive plate through a half-tone screen figure negative to truly reproduce the light tones of the original, repeatedly etching the plate, etching the plate by a plurality of bites and protecting the undercutting made by one bite from the action of a succeeding bite, and removing the resultant roughnesses from the sides of the screen figures of the plate by the application of strong acid.

33. The process of producing a half-tone plate to be used alone in printing, which comprises exposing a light-sensitive plate through a half-tone screen figure negative and creating an enamel design on the surface of the plate, etching the plate by a plurality of bites, and protecting the undercutting made by one bite from the action of a succeeding bite, and removing the resultant roughnesses from the sides of the screen figures of the plate by scrubbing the surface

of the plate with strong acid with all resists removed except the surface enamel.

34. The process of producing a half-tone plate to be used alone in printing, which comprises exposing a light-sensitive plate through a half-tone screen figure negative and creating an enamel design on the surface of a plate, etching the plate, deepening the plate and sharpening and smoothing the screen figures of the plate by scrubbing it with acid with the plate unprotected except by the enamel of the surface design.

35. A half-tone printing plate to be used alone in printing, having the high light dots with smooth sides terminating in points very slightly below the plane of the surface of the plate.

In testimony whereof, we have signed our names to this specification.

AMOS H. SPALDING.

JAMES M. CHANKALIAN.